

## UNITED STATES PATENT OFFICE

2,549,298

## MANUFACTURE OF ACTIVATED CARBON

Joseph W. Donegan, New Brunswick, N. J., assignor to Allied Chemical & Dye Corporation, New York, N. Y., a corporation of New York

No Drawing. Application April 2, 1948,  
Serial No. 18,712

10 Claims. (Cl. 252—421)

1

This invention relates to the manufacture of activatable chars and activated carbons from bituminous materials such as tars and pitches.

Tars and pitches, such as coal tars and water-gas tars and pitches of each, provide a cheap and plentifully available source of raw material for the production of activated carbons suitable for use for decolorizing, deodorizing, and water purification, and also for gas and vapor adsorption purposes. The term "coal tar" as used herein is intended to include all tars resulting from the destructive distillation of coals and typified by such tars as coke oven tar, vertical retort tar, and gas house tar. Conversion of carbonaceous materials into activated carbon normally involves the carbonization or charring of the raw material followed by activation of the resultant char. Previous attempts to use coal tar and water-gas tars and pitches of each as sources of carbon in the manufacture of activated carbon have been unsuccessful chiefly because the pyrolytic cokes resulting from the conventional charring of such materials are essentially non-porous, the pores being so plugged with refractory hydrocarbons as to prevent access of the activating gases to the carbon surfaces, and no prior processes have been developed which adequately take into account these characteristics.

This invention provides methods the practice of which makes commercially feasible the utilization of bituminous raw materials of the types mentioned as sources of carbon for the production of activatable chars and activated carbons. Other objects and advantages of the present improvements will appear from the following detailed description.

A preferred embodiment of the invention involves the production of superior grades of activated carbons from coal tar pitches, and the description of the invention hereinafter given will be confined chiefly to use of these materials, although it is understood that the conditions cited are illustrative and are applicable in principle to any equivalent raw materials.

In accordance with the invention, coal tar, water-gas tar or pitches derived from such tars are treated with a solvent, preferably an aromatic solvent, in such manner as to remove from the tar or pitch a major portion of the benzol-soluble hydrocarbon constituents thereof and obtain a solvent-precipitated pitch product in a finely pulverulent form. This material, containing a major proportion by weight of benzol-insoluble hydrocarbon constituents, is then subjected to

heating in the presence of oxygen-containing gas at temperatures sufficiently high to char the material while maintaining the temperatures sufficiently low during such heating so that at least 5 a substantial proportion of the material remains in unfused condition, and heating of the material is continued until an infusible activatable char is obtained. Preferably: the material subjected to the oxidation treatment is maintained 10 at temperatures above 200° C. during at least the latter stage of charring; the temperature of the material is raised from below 200° C. to within the range of 200—400° C. during the early portion of the charring or oxidation step and is 15 thereafter maintained within the range of 200—400° C. until an infusible activatable char is obtained. In all embodiments of the invention, at the start of the charring operation, the material should not be initially subjected to heating 20 at temperature higher than about 50° C. below the melting point of the particular pitch material being utilized. More particularly, the solvent precipitated material is subjected to an oxidation treatment at slowly increasing temperatures rising from below 200° C. and preferably from below 150° C. to within the range of 200—400° C., preferably to above 300° C., in the presence of a stream of oxygen-containing gas. The rate of temperature rise during this heat treatment must be regulated in accordance with the character of the pitch being processed 25 in order to maintain the temperature below that at which fusion of significant proportions of the hydrocarbons constituting the material occurs, and the heat treatment is continued until an infusible char is obtained. Preferably, the oxygen containing gas above referred to contains from 30 5 to 25% by volume of free oxygen. For example, air, or a flue gas containing about 8% of oxygen, may be employed.

Typical of the suitable raw or starting materials are coal tar pitches. Such pitches contain varying proportions of benzol-insoluble hydrocarbons and benzol-soluble hydrocarbons. 35 Representative coal tar pitches of the type referred to have softening points (cube method) of 30° C. to 220° C., contain from 5% to 60% by weight of benzol-insoluble hydrocarbons, and from 40% to 95% by weight of hydrocarbons 40 which are soluble in benzol. For purposes of this invention, the grade of pitch commercially known as "fuel pitch" has been found particularly suited, pitch of this character having a softening point of 140° C. to 200° C., and containing from 25% to 60% by weight of benzol-

insoluble hydrocarbons. The foregoing benzol-insoluble and benzol-soluble hydrocarbons are likewise respectively insoluble and soluble in other solvents. However, for convenience and purposes of definition, and in accordance with current analytical procedure such hydrocarbons are referred to herein as "benzol-insoluble" and "benzol-soluble."

In carrying out a preferred embodiment of the invention, fuel pitch, after liquefaction if desired, is treated with a suitable solvent, and is thereby separated into high and low melting fractions. In the solvent selected, the high melting fraction (the raffinate) is substantially insoluble and usually contains a major portion of the benzol-insoluble hydrocarbons, while the low melting fraction (the extract) is soluble in the solvent. These fractions then may be separated by any convenient means such as filtration, centrifuging or sedimentation. Satisfactory solvents are predominantly aromatic in character and are typified by the relatively low boiling coal tar distillates boiling within the range of 80° C. to 250° C., such as xylol, benzol, toluol and crude heavy solvent naphthas. The raffinate pitch is characterized by a high melting point and a high content of benzol-insolubles whereas the extracted fraction is low melting and is substantially wholly soluble in benzol, toluol, xylol and similar solvents.

In representative operations, fuel pitch and solvent mixtures are digested and agitated for one or more hours at a temperature of about 90° to 130° C. with about 2 to 10 volumes of solvent per volume of pitch. Type and quantity of solvent employed, extent of agitation, time and temperature of treatment, may be altered within the limits indicated depending upon the desired extent of solution of resins and other aromatic solubles contained in the fuel pitch. In the practice of one method for treating starting material with solvent, a molten coal tar pitch (e. g. 150° C. fuel pitch having 42% benzol insoluble) is cut back by slow addition of one volume of xylol while continuously agitating. This homogeneous cutback pitch is cooled, preferably to about 90° C., and then an additional two volumes of xylol are added, agitation being continued. Dilution with xylol beyond the 1:1 ratio results in a "breaking" of the cutback, or separation into two phases, a liquid continuous phase containing the xylol soluble hydrocarbons, and a solid, finely dispersed solid phase representing those hydrocarbons which are insoluble in the liquor.

In an alternative method for treating starting material, the solid pitch may be digested with approximately three volumes of the solvent used in the former example, the temperature of digestion being approximately 100° C. In this procedure, the soluble bitumens go into solution in the solvent and the insoluble fraction remains in suspension as a finely divided, easily filtered suspensoid. The precipitate formed by either of the foregoing digestion methods may be readily separated from the digestion liquor as by filtration, or otherwise.

The resulting filter cake comprises the high melting, solvent-precipitated pitch together with occluded digestion liquor. Preferably, digestion is regulated to form a fluid mass containing solvent-precipitated hydrocarbon material which, when separated from the solvent liquor by convenient means, contains less than 50% by weight of benzol-soluble hydrocarbons and a major portion by weight of benzol-insoluble hydrocar-

bons. Ordinarily, the above initial digestion yields a filtered precipitated material which may contain approximately 35-40% by weight of benzol-soluble hydrocarbons, although if desired the initial digestion may be carried to a point such that the filtered hydrocarbons contain even lower amounts of benzol-solubles. Particularly in the former instance, further reduction of the benzol-soluble content of the solvent-precipitated pitch and the corresponding increase of the benzol-insoluble content may be easily accomplished by reslurrying or washing the initial digestion stage filter cake with an additional quantity of any one of the suitable solvents, usually the same solvent as used in the primary digestion. If found necessary, the reslurried mass may be kept at temperatures of about 90-100° C. for one or more hours, this procedure effecting extraction of further quantities of the soluble hydrocarbons. Following one or more such additional digestions or washings, the finely pulverulent, precipitated hydrocarbon material containing a substantially smaller amount of associated benzol-soluble hydrocarbons is separated from the warm wash liquor as by filtering.

Whether or not subjected to redigestion or washing to separate additional quantities of hydrocarbons soluble in the solvent employed, the filter cake at hand is dried in any suitable manner, e. g. by heating on trays at temperatures of, say, 90-100° C. in order to evaporate off occluded solvent. Drying should be carried out under such conditions of temperature and time as to avoid any coalescence or possible fusion of the powdered carbonaceous material. While drying, if the temperature is raised too rapidly as the solvent is being eliminated, the solvent will dissolve and flux the pitch, and a fused mass will result. When digestion, washing, and drying are properly carried out as described, the resulting dried intermediate product is a finely pulverulent dust, substantially all passing 325 mesh, and having the below stated compositions and melting points.

In the practice of this invention, the raw material digestion operations, or the combination of primary digestion and the redigestion or washing of the primary digestion stage filter cake, are so carried out or correlated as to produce, after drying, a finely pulverulent, relatively high melting raffinate not less than about 60% of which is insoluble in benzol. Ordinarily, the raffinate is a material not less than about 70% by weight of which is benzol-insoluble and which has a melting point preferably not less than 200° C. In the better embodiments of the invention, digestion, washing and drying are controlled and so effected that the dried raffinate pitch analyzes not less than 75% by weight, and usually more, of benzol-insoluble hydrocarbons and has a melting point desirably not less than 250° C. and preferably not less than 270° C. According to the invention, it has been found that carbonaceous materials having the foregoing characteristics and derived from the starting materials herein disclosed constitute intermediate products which, after selective oxidation in accordance with hereinafter described principles to form infusible chars, are particularly susceptible to activation to produce high-grade activated carbons.

Illustrative of the products formed by the foregoing solvent extraction operations are the following data obtained from the xylol frac-

tionation of a coke oven tar fuel pitch of about 160° C. melting point:

Starting material (160° C. fuel pitch):

Softening point (cube method) °C 160  
Benzol insoluble per cent 32

Extract pitch (after distilling off solvent):

Softening point (cube method) °C 100  
Benzol insoluble per cent 0.6  
Raffinate pitch (oven dried at 100° C.):

Melting point °C 316  
Benzol insoluble per cent 78

"Melting point" as mentioned above and as used herein may be determined by the following procedure: About 50 mm. depth of the pulverulent material is lightly tamped down into a glass tube about 4.0 mm. inside diameter and 75 mm. long which has been sealed off at one end. The filled tube is suspended in an electrically heated air bath and the temperature raised gradually at a rate of about 10° C. per minute, up to the temperature of melting. The melting point is the minimum temperature of the air bath at which powder in the tube shows definite sintering and coalescence of particles.

The next major step of the process is the conversion of the dried, fusible, solvent-precipitated pitch into an infusible char. This conversion is effected by a selective oxidation operation by which the fusible hydrocarbon is converted to an infusible char which is susceptible to activation by known methods. Although the subsequently described selective oxidation may be applied directly to the dried raffinate when it is in the form of a finely pulverulent dust, the dust-like particles may be consolidated in one way or another, and then granulated to afford material of more suitable particle size for further processing. These solvent-precipitated pitches are thermoplastic and therefore do not require addition of binder for subsequent consolidating or briquetting.

The invention provides for the manufacture of activated carbon products suitable for gas and vapor absorption and solvent recovery operations, as well as products adapted for deodorizing and decolorizing. If the final activated product is to be used for gas absorption and/or solvent recovery operations, the dry pulverulent dust is desirably briquetted in compressing machines at pressures ranging from 5,000 to 50,000 pounds per square inch, depending upon the physical structure and density desired in the ultimate product. The briquettes are ground, sized for example to thru 4 on 16 mesh, and the sized material is then subjected to the charring operation. In the manufacture of gas absorption and/or solvent recovery types of activated carbons, briquetting is preferably effected at pressures of e. g. 10,000-40,000 pounds per square inch in such a way as to produce dense briquettes having specific gravities in the range of 1.0-1.3. For production of an activated product particularly suitable for gas masks, pressures of 15,000-25,000 pounds per square inch may be utilized in such manner as to form briquettes having a specific gravity of about 1.2. If the final product is to be used primarily in pulverulent form for treating liquids, the dry dust may be consolidated for example in flaking rolls operating at pressures of, say, 1000 pounds per square inch, the resulting flaked material being ground and sized to form granules, for example through 10 on 60 mesh, and the resulting granules are then subjected to charring.

The charring stage of the invention is effected by subjecting the fusible hydrocarbon precipitate to certain heating and oxidizing conditions. Charring is ordinarily carried out in an externally heated retort, although heating by direct contact with suitable hot gases may be employed. Satisfactory apparatus may comprise a rotary, externally heated retort provided on the inside with agitating flights, equipped on one end with a gas-outlet, and on the opposite end with a gas inlet connected with a suitable metering device and valves so that controlled quantities of an oxidizing gas, e. g. air, may be passed through the retort during the heating operation.

15 The solvent precipitated pitch which is subjected to the charring operation is easily fusible, and the selective oxidation and conversion of this fusible hydrocarbon material to an infusible char is an exothermic reaction. The development work on which the invention is based shows that great care must be taken in effecting the desired conversion to an infusible char, and a major feature of the invention includes the discovery of conditions which make possible such 20 conversion of the fusible hydrocarbon precipitate to an infusible, activatable char. In accordance with this invention, it has been found that the mutually interrelated factors applicable to good embodiments of the invention and upon 25 which accomplishment of the desired result is dependent are the overall heating temperature range; temperature gradient during the entire period of heating; oxygen concentration of the 30 oxidizing gas used during heating; rate of supply of oxidizing gas during the conversion operation; and heating time.

Since the dried hydrocarbon precipitate prior to charring is markedly susceptible to fusion, great care must be exercised throughout the 35 charring operation as a whole, and particularly during the preliminary stages thereof. As previously indicated, the charring reactions are exothermic, and for this reason it is especially necessary to guard against local overheating because, if any of the material is once fused, that portion of the batch is no longer susceptible to activation and either a very low grade of active carbon is produced or the entire batch must be discarded. Prevention of local overheating is largely effected by constant agitation and the passage of gas through the retort throughout the charring run. As the charring of the invention constitutes a selective oxidation, it is also necessary to supply oxygen to the retort.

40 In accordance with the invention, it has been found that adequate amounts of inert gas and oxygen may be supplied to the charring step by passing through the retort, all during the charring stage, a stream of air at a rate within the 45 range of about 1.5-7.5 cu. ft. per 100 pounds of material per minute. It has been found that by utilizing such quantities of air, the oxygen content thereof, i. e. within the range of about 0.3-1.5 cu. ft. per 100 pounds of material per minute, is satisfactory to supply the needed oxygen. Further, the quantity of inert gas in the air along with the oxygen content thereof is enough to maintain in the retort a moving gas stream of sufficient total gas volume to remove the heat of 50 reaction from the mass. While it is preferred to utilize air in the manner stated as the oxidizing-cooling medium, in place of air any gas containing adequate quantities of free oxygen and inert gas may be employed. When using oxidizing gases other than air or its equivalent, for ex-

ample flue gases, such latter gases may contain from 5 to 25% by volume free oxygen, balance inert. Depending upon the free oxygen content of the particular gas used, preferably the gas stream is flowed thru the retort at such a rate that free oxygen is passed thru the retort in quantity within the range of about 0.3-1.5 cu. ft. per 100 pounds of material per minute. Thus, in the case of use of an oxidizing gas containing 5% free oxygen by volume, preferably the gas stream is passed thru the retort at a rate within the range of about 6-30 cu. ft. per 100 pounds of material per minute. In the circumstance of use of a gas containing 25% free oxygen by volume, the gas stream is passed preferably thru the retort at a rate within the range of about 1.2-6.0 cu. ft. per 100 pounds of material per minute.

At the time of introduction into the retort, the precipitated material itself is usually at room temperature or at temperature not higher than the maximum 100-110° C. temperature of drying. Prior to charring, the granular material is in an easily fusible condition. In accordance with the invention, during all of the charring operation temperatures are maintained below temperatures at which fusion of any substantial proportion of the hydrocarbon material would occur. At the beginning of charring, when the granular material is particularly susceptible to fusion, temperatures in the retort are held low. Initially, no portions of the material are heated to temperatures exceeding about 50° C. below the melting point of the particular material being processed. Preferably, initially no portions of the material are heated to temperatures as high as 200° C. Further, in all of the better embodiments of the invention, the material is heated up gradually from a temperature initially not higher than about 150° C. to a temperature of the order of 200° C. This preliminary heating may vary to some extent with respect to both rate of temperature increase and duration. Average rate of temperature increase should be slow, and the temperature gradient may be relatively linear. Duration of preliminary heating may lie within the range of  $\frac{1}{2}$  to 2 hours.

In accordance with the invention, the solvent-precipitated pitch is heated at gradually increasing temperatures from below 200° C., preferably from below 150° C., to within the range of 200-400° C. and in the presence of oxygen-containing gas as above indicated. It has been found e. g. that temperature need not be increased greatly above 200° C., good results having been obtained with maximum temperature of about 250° C. in situations in which time interval of heating is sufficiently extended, e. g. heating at temperature up to about 250° C. for about 8 hours. Ordinarily, temperatures are gradually increased from below 200° C. to within the range of 300-400° C., and in the best embodiments, the gradual heating is carried substantially thru the 200-400° C. range, but temperature should not be permitted to exceed 400° C. Temperature gradient throughout the 200-400° C. range may be relatively linear, and is preferably linear within the 200-300° C. range. Time of heating at temperatures above 200° C. is generally substantially longer than the time interval for heating at temperatures less than 200° C. Duration of heating at temperature above 200° C. may vary from 2 to 8 hours, and is preferably 3 to 8 hours.

Because of variable factors such as the chemical and physical characteristics and properties of the pitch being charred, efficiency of contacting

5 of oxidizing gas and solid material, efficiency of heat dissipation, size of the operation, and the equipment employed, it is not possible to definitely state minimum and maximum heating times which are applicable in all instances. As will be appreciated from the above description and the following examples, various time-temperature cycles are permissible but all have the common requirement that they effect conversion of the fusible hydrocarbon to an infusible char without permitting fusion or leaving incompletely reacted and fusible residues. Thus if a sample of the charred material is heated to 1000° C. and then ground and examined, the presence of brilliant black fused fragments indicates inadequate calcination. Practice of the invention shows that the temperature gradient and total heating time interval sufficient to cause conversion of fusible hydrocarbons to infusible form, i. e. to effect complete charring, may be readily determined on carrying out a few preliminary runs and testing the finally activated products for activity.

20 The charred material may be finally activated by subjecting the same to the action of steam or fine gases, by known procedures, while maintaining temperatures of the general order of 800-1200° C.

25 Examples of practice of the invention are as follows:

*Example 1*

30 A molten coal tar fuel pitch having a softening point (cube in air method) of about 160° C., and containing about 43% by weight of benzoyl-insoluble hydrocarbons and about 57% by weight of benzoyl-soluble hydrocarbons was cut back with an equal volume of industrial xylol. The resultant mass was a smooth homogeneous solution of the pitch which remained fluid at temperatures of about 60-95° C. The solution was then cooled to about 90° C. and a volume of xylol equal to the gross volume of the homogeneous solution was added thereto while stirring continuously. As a result of this dilution, there was precipitated a finely dispersed solid material within the fluid medium. The slurry was filtered, and the insoluble material was obtained as a filter cake analyzing about 66% by weight of benzoyl-insoluble hydrocarbons and about 34% by weight of benzoyl-soluble hydrocarbons. The filter cake 35 was reslurried and washed with another 3 volumes of xylol until there was obtained, after tray-drying at a temperature of about 90° to 100° C., a pulverulent material analyzing about 78% by weight of benzoyl-insoluble hydrocarbons and about 22% by weight of benzoyl-solubles, and having a melting point of about 300° C.

40 This dried, pulverulent pitch product was then briquetted at pressure of about 22,000 lbs. per sq. in., and crushed to thru 10 on 20 mesh, (briquette density—1.20). The thus granulated high density particles were then subjected to selective oxidation in a rotary retort equipped with internal flights, a gas outlet, a metered and valve-controlled gas inlet, and mounted in an electric muffle furnace. The retort was rotated at about 0.2 R. P. M., and the flights in the retort 45 kept the granular material thoroughly agitated. Air was charged into the gas inlet end of the retort so that, throughout the entire run, air was passed into and through the retort at a rate of about 6 cu. ft. per 100 lbs. of material per minute. On introduction into the retort, the material was at about room temperature. Heating by the furnace was so controlled that the temperature 50 of the material in the retort rose to about 200° C.

9

in about one and one-half hours, and then was raised to 300° C. during about three and one-half hours, the rate of increase during this latter interval being substantially linear. The temperature of the material was finally raised to approximately, but not exceeding, 400° C. over a period of about one and one-half hours. Total heating time above 200° C. was five hours.

The resulting char was then activated by treating with steam at about 975° C. in accordance with well established practice.

The superior quality of the improved products is shown by the following data in which two activated carbons of the invention, resulting from the steam activation of chars derived from coal tar fuel pitch and made by runs substantially the same as above described are compared with (#1) a conventional steam activated coconut carbon and (#2) the same coconut carbon further activated with steam in order to attain increased capacity.

| Sample                              | Activated Pitch Carbons | Coco-nut #1 | Coco-nut #2 |
|-------------------------------------|-------------------------|-------------|-------------|
| Sp. Gr. of 12/30 mesh.....          | .500                    | .360        | .500        |
| Service Time—CCl <sub>4</sub> ..... | 18½                     | 19          | 14          |
| Capacity—CCl <sub>4</sub> :         |                         |             |             |
| gms./gm. Carbon.....                | 0.82                    | 1.28        | 0.68        |
| gms./cc. Carbon.....                | 0.41                    | 0.45        | 0.34        |
|                                     |                         |             | 1.08        |
|                                     |                         |             | 0.38        |

The carbon tetrachloride test is that described by Fieldner et al., Industrial and Engineering Chemistry, II, 519 (1919) using air at 25° C. containing 40,000 P. P. M. of carbon tetrachloride.

#### Example 2

A coal tar fuel pitch, obtained by distillation of coke oven tar, having a softening point of about 150° C., and containing about 42% by weight of benzol-insoluble hydrocarbons and about 58% by weight of benzol-soluble hydrocarbons was pulverized and digested with about 2½ volumes of xylol for 2 hours at a temperature of about 90–130° C. The slurry was filtered, and the insoluble material was obtained as a filter cake containing about 30% by weight of benzol-soluble hydrocarbons. The filter cake was reslurried and washed with another 2½ volumes of xylol, and there was obtained, after tray drying at about 110° C., a pulverulent pitch containing about 77% by weight of benzol-insoluble hydrocarbons and about 23% by weight of benzol-solubles, and having a melting point of about 295° C.

The dried powder was then briquetted at pressure of about 20,000 lbs. per sq. in., and crushed to through 6 on 20 mesh. The thus granulated material was then subjected to selective oxidation in a rotary retort of the type of Example 1. The retort was rotated at about 0.2 R. P. M., and the flights in the retort kept the granular material thoroughly agitated. Air was charged into the gas inlet end of the retort so that, throughout the entire run, air was passed into and through the retort at a rate of about 6 cu. ft. per 100 lbs. of material per minute. On introduction into the retort, the material was at about room temperature. The heating cycle was substantially the same as that of Example 1. The resulting carbonaceous char was then activated with steam in accordance with known procedure at temperature of about 975° C. to a weight loss of about 60%. A 0.25 gram sample of the product, crushed to pass a 200 mesh screen, adsorbed 92% of the iodine from a standard iodine solution. The activated material, when crushed to thru

10

12 on 16 mesh, had a bulk density of 0.500 and, when exposed to an atmosphere containing 40,000 P. P. M. of carbon tetrachloride at 25° C., adsorbed 85% of its own weight of carbon tetrachloride. Heat of wetting by benzene was 23 calories per gram. Similar activation of another portion of the same granular char thru 6 on 20 mesh activated to a weight loss of 75% gave a product which had a bulk density of 0.400, a heat of wetting by benzene of 26 calories per gram, and a carbon tetrachloride capacity of 120% of its own weight. The granular products described may be ground in suitable apparatus if a finely pulverized grade of carbon be desired.

#### Example 3

A flaked fuel pitch obtained by vacuum distillation of water gas tar and which was characterized by a softening point of about 150° C. and a benzol-insoluble content of 31%, was extracted by digesting with 3 volumes of a crude solvent naphtha boiling within the range of 125 to 250° C. Digestion was effected by adding the cold pitch to the cold solvent and agitating continuously while raising the temperature to 90° C. over a one-hour period. The resultant slurry was filtered, and the cake was washed with an additional 3 volumes of the solvent so that there was obtained, after drying at about 100° C., a carbonaceous product comprising approximately 80% benzol-insoluble hydrocarbons and 20% benzol-soluble components. The melting point of this product was about 310° C.

The pulverulent pitch product was lightly compacted by passing thru a differential speed roll mill and the resultant flake was granulated to provide low density grain of 10 to 20 mesh size. Calcination for conversion into a suitable infusible char was carried out by heating in the apparatus of the preceding examples. On introduction into the retort, the material was at about room temperature. However, in this operation, instead of air, a flue gas containing 10% oxygen was passed through the retort at the rate of about 10 cu. ft. per 100 lbs. of material per minute. The heating cycle followed was substantially the same as that of Example 1, and a well-calcined char was produced.

After calcination, the char was activated by heating to 1100° C. while passing carbon dioxide thru the retort. The activated product, representing 30% of the char, was of such activity that 0.5 gram removed 91% of the color from a standard brown sugar solution. A high grade of commercial decolorizing carbon removed 88% of the color in a comparable test.

#### Example 4

A coke oven tar fuel pitch was produced by air blowing a residuum of 66° C. softening point until the product had a softening point of 219° C. and a benzol-insoluble content of 50%. This pitch was fractionated by extraction of the pulverized pitch with 5 volumes of crude solvent naphtha boiling within the range of 125 to 250° C. The precipitated hydrocarbons required no washing and, after filtration and drying, were obtained as a dry, pulverulent solid material melting above 350° C. and analyzing 86% benzol-insoluble.

The low solubility and refractory nature of this hydrocarbon made possible a very rapid oxidation. After briquetting to 1.20 block density and granulation to 10–20 mesh size, the material was charged, at about room temperature, into the retort of Example 1. Conversion to a satisfactory

## 11

char was effected on the following heating cycle: One and one-half hours to 200° C., two hours from 200 to 300° C., and one hour from 300 to 400° C. Throughout the calcination, air was passed through the retort at the rate of about 6 cu. ft. per 100 lbs. of material per minute.

The calcination product was adequately charred and completely infusible. After activation with steam at 1000° C. to 60% weight loss, the grain had a carbon tetrachloride service time of 20 minutes, a capacity of .820 gram CCl<sub>4</sub> per gram of carbon, and a heat of wetting with xylol of 23 calories per gram.

## Example 5

Precipitated pitch hydrocarbon, obtained from the same coal tar fuel pitch, by substantially the same extraction procedure, and having substantially the same properties, all as in Example 2, was briquetted at 20,000 lbs. per sq. in. and then granulated to 10-20 mesh size. The resultant material was charged into the retort of Example 1. The retort was rotated at about 0.2 R. P. M., and the flights in the retort kept the granular material thoroughly agitated. Air was charged into the gas inlet end of the retort so that, throughout the entire run, air was passed into and through the retort at a rate of about 3 cu. ft. per 100 lbs. of material per minute. On introduction into the retort, the material was at about room temperature. The temperature was raised to 200° C. in one hour, and then gradually raised to about 250° C. over a period of about 8 hours. The material was completely converted to an infusible char, and on activation with steam at 1000° C., yielded a product giving 20 minutes service time in the CCl<sub>4</sub> test.

The benzol-insoluble contents and cube melting and softening points of the materials referred to herein are determined by standard tests prescribed in "Methods of Testing Coal-Tar Products" (revised July 1942), published by The Barrett Division, Allied Chemical & Dye Corporation, 40 Rector Street, New York, copyright Allied Chemical & Dye Corp. 1931 and 1942.

I claim:

1. The process for making an activatable char from a solid carbonaceous material containing not less than 60% by weight of benzol-insoluble constituents derived from starting material of the group consisting of coal tar and water-gas tar and pitches of each, which comprises heating said derived carbonaceous material at increasing temperatures from below 200° C. to within the range of 200°-400° C. in the presence of free oxygen-containing gas, the free oxygen concentration of said gas being sufficiently high to selectively oxidize and convert said carbonaceous material to an infusible char, maintaining the temperatures of said carbonaceous material during heating below temperatures at which fusion of a substantial proportion of the carbonaceous material would occur, and continuing heating until an infusible activatable char is obtained.

2. The process for making an activatable char which comprises extracting hydrocarbon material of the group consisting of coal tars, water-gas tars and their pitches with a predominantly aromatic solvent to produce hydrocarbon material containing not less than 70% by weight of benzol-insoluble constituents, heating said last-named hydrocarbon material at gradually increasing temperatures from below 200° C. to within the range of 200°-400° C. in the presence of free oxygen-containing gas, the free oxygen

## 12

concentration of said gas being sufficiently high to selectively oxidize and convert said last-named hydrocarbon material to an infusible char, maintaining the temperatures of said material throughout said heating period below temperatures at which fusion of a substantial proportion of the hydrocarbons constituting the material would occur, and continuing said heat treatment until an infusible activatable char is obtained.

3. The process for making an activatable char from a solid carbonaceous material containing not less than 70% by weight of benzol-insoluble constituents and having a melting point not less than 200° C. and derived from starting material

15 of the group consisting of coal tars, water-gas tars and their pitches, said process comprising heating said derived carbonaceous material at gradually increasing temperatures from below 200° C. to within the range of 200°-400° C. in the presence of a gas containing 5-25% by volume free oxygen, maintaining the temperature of the thus heated material at all times throughout said heating period below the temperature at which 20 fusion of a substantial proportion of the solids present in said material at that time would occur, and continuing said heating above 200° C. 25 until an infusible activatable char is obtained.

4. The process for making an activatable char 30 which comprises extracting hydrocarbon material of the group consisting of coal tars, water-gas tars and their pitches with a predominantly aromatic solvent to produce hydrocarbon material in a finely pulverulent form and containing 35 a major portion by weight of benzol-insoluble hydrocarbons and having a melting point not less than 200° C., heating said last-named hydrocarbon material at gradually increasing temperatures from below 200° C. to within the range 40 of 200°-400° C. in the presence of a gas containing at least 5% by volume free oxygen, maintaining the temperatures of said material throughout said heating period below temperatures at which fusion of a substantial proportion 45 of the hydrocarbons constituting the material would occur, and continuing said heat treatment until an infusible activatable char is obtained.

5. The process for making an activatable char 50 which comprises forming a solid material containing not less than 70% by weight of benzol-insoluble hydrocarbons, having a melting point not less than 200° C. and derived from starting material of the group consisting of coal tar and water-gas tar and pitches of each, heating said solid material at gradually increasing temperatures from below 200° C. to within the range of 200°-400° C., carrying out said gradual heating 55 operation, substantially thru said 200°-400° C. range but to temperature not exceeding 400° C., 60 in the presence of a gas containing 5-25% by volume free oxygen, maintaining the temperatures of said material throughout said heating period below temperatures at which fusion of a substantial proportion of the hydrocarbons constituting the material would occur, and continuing said heat treatment until an infusible activatable char is obtained.

6. The process for making an activatable char 65 which comprises forming a solid material containing not less than 70% by weight of benzol-insoluble hydrocarbons and derived from starting material of the group consisting of coal tar and water-gas tar and pitches of each, heating said solid material at gradually increasing 70 temperatures from below 200° C. to within the range 75

of 200°-400° C., carrying out said gradual heating operation while agitating and while passing thru said agitated material a stream of a gas containing at least 5% by volume free oxygen at a rate such as to pass thru said material free oxygen within the range 0.3-1.5 cu. ft. per 100 lbs. of material per min., and continuing said heating operation for a time interval sufficient to effect conversion of said material to an infusible activatable char.

7. The process for making an activatable char which comprises forming a solid material containing not less than 70% by weight of benzol-insoluble hydrocarbons, having a melting point not less than 200° C. and derived from starting material of the group consisting of coal tar and water-gas tar and pitches of each, heating said solid material in granular form at gradually increasing temperatures from below 200° C. to within the range of 200°-400° C., carrying out said gradual heating operation (1) substantially thru said 200°-400° C. range but to temperature not exceeding 400° C., (2) while agitating, and (3) while passing thru said agitated material a stream of a gas containing at least 5% by volume free oxygen at a rate such as to pass thru said material free oxygen within the range 0.3-1.5 cu. ft. per 100 lbs of material per min., and continuing said heating operation for a time interval sufficient to effect conversion of said material to an infusible activatable char.

8. The process for making an activatable char which comprises forming a solid material containing not less than 70% by weight of benzol-insoluble hydrocarbons, having a melting point not less than 200° C., and derived from starting material of the group consisting of coal tar and water-gas tar and pitches of each; heating said solid material in granular form at gradually increasing temperatures from below 200° C. to within the range of 200°-400° C., carrying out said gradual heating operation (1) substantially through said 200°-400° C. range but to temperature not exceeding 400° C., (2) while agitating, and (3) while passing through said agitated material a gas stream, containing 5-25% by volume free oxygen, at a rate such as to pass through said material free oxygen within the range 0.3-1.5 cu. ft. per 100 lbs. of material per min., and continuing said heating operation above 200° C. for a time interval within the range of 2-8 hours and sufficient to effect conversion of said material to an infusible activatable char.

9. The process for making activated carbon which comprises forming a solid material containing not less than 75% by weight of benzol-insoluble hydrocarbons, having a melting point not less than 250° C., and derived by solvent precipitation from starting material of the group consisting of coal tar and water-gas tar and pitches of each, heating said solid material in granular form at gradually increasing temperatures from below 150° C. to within the range of 200°-400° C., carry-

ing out said gradual heating operation (1) substantially through said 200°-400° C. range but to temperature not exceeding 400° C., (2) while agitating, and (3) while passing thru said agitated material a stream of air at a rate within the range 1.5-7.5 cu. ft. per 100 lbs. of material per min., continuing said heating operation above 200° C. for a time interval within the range of 2-8 hours and sufficient to effect conversion of said material to an infusible activatable char, and then subjecting the thus heat treated material to the action of carbon activating medium at temperature above 800° C.

10. The process for making a hard dense activated carbon adaptable for vapor absorption which comprises extracting coal tar fuel pitch having a softening point of about 140°-200° C. with a predominantly aromatic solvent boiling within the range of 80°-250° C., carrying out the 15 treating operation in the presence of a sufficient quantity of solvent and under conditions to effect solution by the solvent of at least the major portion of the benzol-soluble hydrocarbons contained in said material and to effect formation of 20 a precipitate containing benzol-insoluble hydrocarbons, recovering from the solvent liquor dry, pulverulent material containing not less than 75% by weight of benzol-insoluble hydrocarbons and having a melting point not less than 250° C., compressing the material under pressure sufficient to 25 form dense briquettes having specific gravity in the range of 1.0-1.3, heating said briquetted material in granular form at gradually increasing temperatures from below 150° C. to within the 30 range of 200°-400° C., carrying out said gradual heating operation (1) substantially through said 200°-400° C. range but to temperature not exceeding 400° C., (2) while agitating, and (3) while 35 passing thru said agitated material a stream of air at a rate within the range 1.5-7.5 cu. ft. per 100 lbs. of material per min.; continuing said heating operation above 200° C. for a time interval within the range of 2-8 hours and sufficient to 40 effect conversion of said material to an infusible 45 activatable char, and then subjecting the thus heat treated material to the action of carbon activating medium at temperature above 800° C.

JOSEPH W. DONEGAN.

#### REFERENCES CITED

The following references are of record in the file of this patent:

#### UNITED STATES PATENTS

| 55 | Number    | Name         | Date           |
|----|-----------|--------------|----------------|
|    | 1,553,641 | Sperr _____  | Sept. 15, 1925 |
|    | 1,731,473 | Naugle _____ | Oct. 15, 1929  |

#### OTHER REFERENCES

|    |                                                                            |
|----|----------------------------------------------------------------------------|
| 60 | Deitz: "Bibliography of Solid Adsorbents," page 776, 2nd paragraph (1944). |
|    | British Chemical Abstracts-B, pages 1098-9 (1930).                         |